

# United States Patent

Brown et al.

[15] 3,660,177

[45] May 2, 1972

[54] **PROCESSING OF NICKEL-BASE ALLOYS FOR IMPROVED FATIGUE PROPERTIES**

[72] Inventors: **Edgar E. Brown, Glastonbury; Raymond C. Boettner, Windsor, both of Conn.**

[73] Assignee: **United Aircraft Corporation, East Hartford, Conn.**

[22] Filed: **May 18, 1970**

[21] Appl. No.: **38,227**

[52] U.S. Cl. .... **148/11.5 R, 148/11.5 F, 148/12.7**

[51] Int. Cl. .... **C22f 1/10**

[58] Field of Search..... **148/11.5 R, 11.5 F, 12.7**

[56]

**References Cited**

**UNITED STATES PATENTS**

3,519,503 7/1970 Moore et al. .... **148/11.5 F**  
3,420,716 1/1969 Slepitis..... **148/11.5 R**

*Primary Examiner*—Richard O. Dean

*Attorney*—Richard N. James

[57] **ABSTRACT**

The fatigue properties of the precipitation-hardened, nickel-base alloys, such as Inconel 718, Incoloy 901 and Waspaloy, are significantly improved by a thermomechanical processing technique involving the generation of an intermetallic pinning phase, such as a spheriodal eta phase or an overaged gamma prime phase, with subsequent recrystallization to provide a uniform microstructure having a grain size of ASTM 10-13 or finer.

**11 Claims, 4 Drawing Figures**



PATENTED MAY 2 1972

3,660,177

SHEET 1 OF 2

FIG. 3



FIG. 2



FIG. 1





## PROCESSING OF NICKEL-BASE ALLOYS FOR IMPROVED FATIGUE PROPERTIES

### BACKGROUND OF THE INVENTION

The present invention relates in general to the nickel-base alloys and, more particularly, to a novel fabrication process therefor to provide improved physical properties including increased fatigue resistance.

In the gas turbine engine industry where so many of the strong nickel-base alloys have great utility, experience has demonstrated that one of the critical factors which must be considered is the fatigue resistance of the alloys. For gas turbine engine disks and shafts, fatigue resistance, particularly low cycle fatigue resistance, may in fact be the limiting factor in the establishment of the useful operating lives of such components. Although the fatigue problem may in some instances be solved by the substitution of other materials or by alterations in alloy chemistry, such substitutions or alterations are usually made with considerable reluctance, usually for economic reasons although the drawbacks incident to the development of new experience factors with new alloys or old alloys in new applications are also of importance.

It is well known that the physical properties of engine components are dependent not only upon their alloy chemistries but also upon their fabrication histories. With proper processing specific alloys may be provided with specific property alterations or the alloy properties may in general be enhanced. One such improved processing technique is disclosed in the copending application of G. H. Rowe et al. entitled "Process for Improving the Fatigue Resistance of Certain Nickel-Base Alloys," application Ser. No. 775,541, filed Nov. 13, 1968 and assigned to the present assignee. Another advanced processing technique applicable to the nickel-base superalloys is that described in the copending application of W. A. Owczarski et al. entitled "Thermomechanical Strengthening of the Superalloys," application Ser. No. 864,268, filed Sept. 26, 1969 and also assigned to the present assignee.

Of particular interest in the present process are those nickel-base alloys of the type typified by Inconel 718, Incoloy 901 and Waspaloy, representative chemistries for these alloys being as follows:

|        | Inconel 718 | Incoloy 901 | Waspaloy             |
|--------|-------------|-------------|----------------------|
| Ni     | Balance     | Balance     | Balance              |
| Cr     | 18.5        | 12.5        | 19.5                 |
| Co     | —           | —           | 13.5                 |
| C      | 0.1         | 0.1         | 0.08                 |
| Fe     | 18          | 34          | —                    |
| Ti     | 0.9         | —           | 3                    |
| Al     | 0.6         | 2.6         | 1.4                  |
| Mo     | 3           | 6           | 4                    |
| Others | 5 (Cb+Ta)   | 0.015 (B)   | 0.005(B)<br>0.08(Zr) |

### SUMMARY OF THE INVENTION

This invention contemplates the processing of certain precipitation hardened nickel-base alloys to provide improved fatigue resistance thereto. It is applicable to those nickel-base alloys precipitating intermetallic compounds, such as an eta ( $Ni_3Cb$ ,  $Ni_3Ti$ ) or overaged gamma prime ( $Ni_3Al$ , Ti), which are stable above the alloy recrystallization temperature and which may be produced in the microstructure below the alloy recrystallization temperature. These are hereinafter collectively referred to as pinning phases.

In the fabrication sequence, the alloys are thermodynamically processed to provide a uniform dispersion of a fine pinning phase and subsequently recrystallized. The uniform dispersion of the pinning phase may be provided in a number of ways including: cold or warm working the alloy and subsequently heat treating the as-worked structure to precipitate a spheroidal eta or overaged gamma prime phase; warm working at a temperature sufficient to induce precipitation of the pinning phase during deformation; or establishment of a con-

ventional needle-like eta phase and subsequent thermomechanical processing to effect a conversion to the desired pinning phase such as the fine spheroidal eta.

In the more preferred processing sequence for the alloys capable of eta precipitation, the alloy is first subjected to heat treatments to minimize alloy heterogeneity and to precipitate the conventional needle-like eta; then warm worked to effect a conversion of the eta to a uniform fine dispersion of the desired spheroidal eta; and subsequently recrystallized to form a microstructure having a grain size of ASTM 10-13 or finer. Normally, the conventional aging heat treatments are thereafter applied for strengthening purposes.

### BRIEF DESCRIPTION OF THE DRAWINGS

FIG. 1 is a photomicrograph of conventionally processed Inconel 718 bar stock revealing a comparatively coarse grain size (ASTM 4-5) with the absence of any significant amount of the eta phase. (150 $\times$ before reduction).

FIG. 2 is a photomicrograph of an Inconel 718 pancake processed according to the present invention and illustrating a fine grain size (ASTM 12). (250 $\times$ before reduction).

FIG. 3 is a photomicrograph, at greater magnification, of the sample of FIG. 2 showing a uniform distribution of spherical eta particles refining grain size. (1,000 $\times$ before reduction).

FIG. 4 is a graph plotting the fatigue resistance of Incoloy 901 as a function of grain size.

### DESCRIPTION OF THE PREFERRED EMBODIMENTS

The demands for improved engine performance and increases in engine operating temperatures, and product improvement programs designed to increase the operating lives of engine components have progressed to the point where material's limitations have been reached. In particular, gas turbine engine shafts and disks have been found to be limited by low cycle fatigue in many instances. In the study of the fatigue behavior of certain nickel-base alloys as a function of heat treatment, it was determined that ultra-fine grain sizes can provide vastly improved fatigue and strength properties. It was further determined that by suitable processing, the grain size can be substantially reduced by the precipitation of particular intermetallic pinning phases prior to recrystallization.

In the case of Inconel 718, grain size refinement can be achieved through precipitation of an eta phase prior to recrystallization. Eta in this alloy is an orthorhombic  $Ni_3Cb$  phase which is typically precipitated in this alloy in the 1,600°-1,700° F. temperature range and which is stable above the alloy recrystallization temperature. Normally, as eta is allowed to precipitate in fully annealed alloy, it nucleates at grain boundaries and grows preferentially along (111) crystallographic planes, forming long straight needles traversing each grain. Inasmuch as in this form it does not contribute significantly to the strength of the alloy and in fact competes for the elements forming the hardening gamma prime precipitate, most of the literature has concluded that the eta phase should be avoided.

If, however, the eta precipitate is forced to precipitate in a material which has been deformed below the alloy recrystallization temperature or otherwise properly processed, it may be provided in a uniform dispersion throughout the matrix, appearing metallographically as generally spheroidal particles 1-3 microns in size. This may be seen in FIG. 3. If the alloy is then recrystallized with the uniform dispersion of fine spheroidal eta present, the newly formed grain boundaries incorporate the eta, effectively inhibiting grain growth. The result is a much finer, more uniform grain size than that achieved by conventional processing, which may readily be observed by a comparison of the microstructures of FIGS. 1 and 2. Early indications revealed that with proper processing the grain size could be reduced from ASTM 3 to at least about ASTM 10 with an increase in fatigue resistance of about 40 percent. It is therefore now possible to provide nickel-base alloys having fatigue strengths equal to or exceeding those attainable in the

iron-base alloy systems wherein the fatigue properties are often independent of grain size.

The significant property improvements have been obtained only in those nickel-base alloys displaying the fine grain size which, in turn, is a function not only of the heat treatments but of the entire processing parameters and sequencing. For reproducibility and the attainment of optimum results, stringent control over the entire fabrication process is mandatory, including close control of the forging or other deformation variables.

Experience has demonstrated that a number of criteria must be satisfied for effective results. The pinning precipitate must be stable at temperatures in excess of the alloy recrystallization temperature for the grain refining function of the precipitate depends, of course, on its presence during the recrystallization process. The pinning precipitate must precipitate profusely at temperatures below the recrystallization temperature and it must be dispersed uniformly throughout the microstructure. And recrystallization must occur subsequent to the formation and dispersion of the pinning precipitate. For practical reasons in production runs, a reasonable spread between the recrystallization temperature and the solvus temperature of the pinning precipitate is very much preferred as hereinafter discussed in greater detail.

The Incoloy 901 alloy exhibits precipitation of a hexagonal  $Ni_3Ti$  eta phase with characteristics similar to the  $Ni_3Cb$  phase observed in Inconel 718. Retardation of grain growth by a uniform dispersion of spheroidal eta has also been accom-

The present processing has also been applied to Waspaloy wherein the grain growth retardation function during recrystallization is provided by an overaged gamma prime precipitate. This pinning precipitates, having an average diameter of 0.5-1 micron, are introduced into the material prior to forging or other deformation by a heat treatment of 1,800°-1,825° F. for 24-48 hours.

Recrystallization is a process whereby cold-worked material reverts to a strain-free structure by the nucleation and growth of new grains. In the precipitation hardened, nickel-base alloys recrystallization is conducted above the solvus temperature of the hardening phase or phases. In the Inconel 718 and Incoloy 901 alloys, the pinning eta precipitate and the hardening gamma prime phase are characterized by divergent solvus temperatures and recrystallization is conducted at a temperature above the gamma prime solvus but below that of the pinning phase. In the case of Waspaloy as conventionally formulated, the pinning precipitate and the hardening phase are essentially identical chemically and metallurgically, the primary difference residing in the size of the precipitate. However, because of this size difference, it is possible to solution the hardening phase while retaining the effect of the overaged precipitate for grain size control, since the smaller particles are more readily solutioned. However, the recrystallization process is time-limited in this alloy.

Table II compares the precipitation characteristics of the eta and the gamma prime hardening phases in the Inconel 718 and Incoloy 901 alloys.

TABLE II  
[Comparison of the Pinning and Hardening Precipitation Reactions]

| Phase       | Chemical composition                                | Crystallographic structure | Approximate particle size  | Precipitation temperature range typical | Maximum stability temperature         | Strengthening characteristics  |
|-------------|-----------------------------------------------------|----------------------------|----------------------------|-----------------------------------------|---------------------------------------|--------------------------------|
| Eta         | { $Ni_3Cb$ (Inconel 718)<br>$Ni_3Ti$ (Incoloy 901)} | Orthorhombic.....          | 10,000-20,000 <sup>1</sup> | 1,800°-1,750° F.                        | { 1,800° F. (718)<br>1,750° F. (901)} | None.                          |
|             | { $Ni_3Cb$ (718)<br>$Ni_3Ti$ (901)}                 | Hexagonal.....             |                            |                                         |                                       |                                |
| Gamma prime | { $Ni_3Ti$ (901)<br>$Ni_3(A_1, Ti)$ (Wasp)}         | Face centered.....         | 300-500 Å. <sup>2</sup>    | 1,000°-1,500° F.                        | 1,700°-1,800° F.                      | Major strengthening mechanism. |
|             | { $Ni_3(A_1, Ti)$ .....                             | Cubic.....                 |                            |                                         |                                       |                                |
| Overaged    |                                                     | Face centered.....         | 0.5-1 micron.....          | 1,775-1,860° F.                         | 1,850° F.                             | Limited strengthening.         |
| Gamma prime |                                                     | Cubic.....                 |                            |                                         |                                       |                                |

<sup>1</sup> Visible optically.

<sup>2</sup> Not visible optically.

plished with this alloy. As compared to conventionally processed Incoloy 901, the fine grain structures processed according to the present invention exhibiting grainsizes of ASTM 10 (0.0002 inch diameter) or finer display superior fatigue and tensile strength properties. Tensile and yield strengths are increased by a factor of about 10-20 percent, and the smooth high cycle fatigue (HCF) life is increased by a factor of 40 percent.

In its chemistry, Incoloy 901 does present somewhat of a practical processing problem. Whereas Inconel 718 exhibits a 50°-75 F. temperature differential between the eta solvus and the recrystallization temperature, the differential for Incoloy 901 is only about 15°-25° F. Due to this very narrow differential, processing difficulties are increased with these alloys. It is, of course, possible to resolve this problem by certain modifications in alloy composition. Eta solvus temperatures were determined for several such modifications as detailed in Table I.

TABLE I

| Sample | Eta solvus       | C   | Cr   | Mo  | Ti  | B    | Ni | Fe   |
|--------|------------------|-----|------|-----|-----|------|----|------|
| 1*     | 1,775° 1,800° F. | .03 | 13.5 | 5.5 | 2.9 | .015 | 45 | Bal. |
| 2      | 1,900° 1,925° F. | .03 | 15.6 | 7.1 | 4   | .015 | 45 | Bal. |
| 3      | 1,875° 1,900° F. | .03 | 13.5 | 7.1 | 4   | .015 | 45 | Bal. |
| 4      | 1,825° 1,860° F. | .03 | 11.5 | 7.1 | 4   | .015 | 45 | Bal. |
| 5      | 1,825° 1,860° F. | .03 | 13.5 | 5.5 | 4   | .015 | 45 | Bal. |

\*Control composition.

Increasing chromium, molybdenum and titanium contents result in higher eta solvus temperatures, and for all compositions the recrystallization temperature appears to be below 1,775° F. These modified alloys can be forged to the desired fine grain condition at higher forging temperatures and over a wider temperature range than the control composition.

As indicated in Table II, eta precipitates in the Inconel 718 and Incoloy 901 alloys at the nominal chemistry in the 1,500°-1,700° F. range. If fully annealed material is exposed to heat treatment in this temperature range, eta precipitation will occur as a needle-like phase whereas the desired grain size refinement is dependent upon the presence of eta as a uniform distribution of spheroidal particles.

Spheroidal eta precipitation may be caused to occur under either of two processing conditions: (1) heat treatment of cold worked alloys of this type in the 1,600°-1,700° F. temperature range, or (2) warm working below the recrystallization temperature (1,750° F.). In addition, spheroidal eta may be provided by warm working the alloys containing the needle-like eta below the alloy recrystallization temperature.

The extent of working is not critical as long as sufficient energy for recrystallization is imparted to the structure to provide spheroidal eta precipitation with these alloys. Room temperature deformation of Inconel 718 will generally exceed about a 40 percent reduction in thickness and that for Incoloy 901 a 50 percent reduction to ensure spheroidal eta precipitation upon subsequent heat treatment.

In the case of Waspaloy, an overaged gamma prime precipitate is introduced into the material by a heat treatment at 1,800°-1,825° F. for 24-48 hours. Because the precipitate so formed is large and incoherent compared to the hardening gamma prime that is produced during aging (1,400° F.), the hardness of the material is relatively low. Subsequent working operations to the desired configuration (typically hammer forging, press forging or extrusion) at 1,800°-1,850° F. will provide the desired recrystallization energy at reductions of 30 percent.

The preferred processing conditions for the Inconel 718 and

Incloy 901 alloys is as follows: (a) homogenization, and eta precipitation heat treatment at 1,650°-1,700° F. for 4-8 hours, (b) forging at a 50-65 percent reduction at or below the eta solvsus temperature (1,825° F. and 1,750° F., respectively, for the above alloys) and (c) solution heat treatment with recrystallization 25°-50° F. below the eta solvsus. The latter heat treatment for 1 hour is sufficient to induce recrystallization without substantial grain growth. Short time reheats in excess of those described are tolerable provided that the eta structure is not adversely affected and no substantial grain growth occurs.

After establishment of the grain size as above described, the alloys prior to use are subjected to the usual aging heat treatment for strengthening through precipitation of the hardening gamma prime phase. For Inconel 718, this comprises holding at 1,325° F. for 8 hours, and 1,150° F. for 8 hours. For Incloy 901, the aging comprises heat treatment at 1,325° F. for 6 hours and 1,200° F. for 12 hours. Cooling rates are generally equivalent to air cool or faster.

With Waspaloy the preferred processing involves: (a) an initial heat treatment at 1,800°-1,825° F. for 24-48 hours to form the overaged gamma prime precipitate; forging to the desired configuration using a preheat temperature of 1,800°-1,850° F. and reductions of 30 percent or more; and heat treatment at 1,800°-1,850° F. for 2-4 hours for recrystallization, providing a grain size of ASTM 10 or finer. A sustained temperature of 1,850° F. cannot be exceeded during any stage of the process subsequent to the formation of the overaged gamma prime pinning precipitate because of its instability above this temperature. A final stabilization heat treatment at about 1,550° F. for 4 hours and aging at about 1,400° F. for 16 hours will provide a full hardness response.

The property improvements incident to the preferred processing according to this invention may be seen from FIG. 4 of the drawings and the following tables.

TABLE III  
[Tensile and high cycle fatigue properties of Inconel 718 barstock material processed to several grain sizes. All data recorded at 850° F.]

| Grain size   | Fatigue strength, K.s.i. | Ultimate tensile strength, K.s.i. | 0.2% yield strength, K.s.i. | Elongation, percent | Fatigue ratio FS/UTS |
|--------------|--------------------------|-----------------------------------|-----------------------------|---------------------|----------------------|
| ASTM 13..... | 114                      | 193                               | 158                         | 22.5                | 0.60                 |
| ASTM 10..... | 97                       | 177                               | 151                         | 21.5                | 0.54                 |
| ASTM 5.....  | 80                       | 170                               | 154                         | 17.5                | 0.47                 |
| ASTM 3.....  | 55                       | 166                               | 144                         | 20.0                | 0.33                 |

LCF data on fine grain Inconel 718 barstock material

| Grain size   | Stress, K.s.i. | Temperature, °F. | Cycles to failure (avg.) |
|--------------|----------------|------------------|--------------------------|
| ASTM 12..... | 30±65.5        | 850              | 1200,000                 |
| ASTM 12..... | 40±80          | 1,000            | 41,000                   |

Stress rupture data on fine grain Inconel 718 barstock material

| Grain size   | Stress, K.s.i. | Temperature, °F. | Time to rupture, hours | R.T. elongation, percent |
|--------------|----------------|------------------|------------------------|--------------------------|
| ASTM 10..... | 90             | 1,200            | 203.1                  | 13.1                     |
| ASTM 13..... | 90             | 1,200            | 170.6                  | 12.8                     |
| ASTM 10..... | 75             | 1,300            | 27.4                   | 16.9                     |
| ASTM 13..... | 75             | 1,300            | 14.1                   | 22.1                     |

1 No failure.

TABLE IV  
[Comparison of LCF properties of fine grain Incloy 901 with conventionally processed Incloy 901 materials]

| Alloy           | Grain size   | Stress, K.s.i. | Temperature, °F. | Cycles to failure |
|-----------------|--------------|----------------|------------------|-------------------|
| Incloy 901..... | ASTM 12..... | 30±65.5        | 850              | 1200,000          |
|                 | ASTM 5.....  | 30±65.5        | 850              | 20,000-49,000     |
|                 | ASTM 2.....  | 30±65.5        | 850              | 2,000-15,000      |
|                 | ASTM 12..... | 30±77.5        | 850              | 127,000-147,000   |

Table IV - Continued  
[Comparison of LCF properties of fine grain Incloy 901 with conventionally processed Incloy 901 materials]

| Alloy                                                           | Grain size   | Stress, K.s.i. | Temperature, °F. | Cycles to failure     |
|-----------------------------------------------------------------|--------------|----------------|------------------|-----------------------|
|                                                                 | ASTM 5.....  | 30±77.5        | 850              | 11,000-35,000         |
| Stress rupture data for fine grain Incloy 901 barstock material |              |                |                  |                       |
| 10                                                              | Grain size   | Stress, K.s.i. | Temperature, °F. | Time to rupture, hrs. |
|                                                                 | ASTM 12..... | 90             | 1,200            | 12.8                  |
|                                                                 | ASTM 12..... | 80             | 1,200            | 37.2                  |

15 1 No failure.

Thus, by providing a fine uniform dispersion of a pinning precipitate, such as the spheroidal eta phase or the overaged gamma prime, prior to recrystallization, and effecting recrystallization in the presence of the pinning phase to control the grain size, it is possible to provide dramatic improvements in the fatigue resistance of nickel-base alloys of the type typified by Inconel 718, Incloy 901 and Waspaloy.

20 Although the invention has been described in detail with reference to certain preferred embodiments and examples for the purpose of illustration and explanation, the invention in its broader aspects is not limited to the exact details described, but improvements to and departures therefrom may be made 25 within the scope of the appended claims without departing from the principles of the invention and without sacrificing its chief advantages.

30 What is claimed is:

35 1. The method of improving the fatigue resistance of the precipitation hardenable, nickel-base alloys capable of precipitating intermetallic compounds which are stable above the alloy recrystallization temperature which comprises: 40 thermomechanically processing the alloy to develop a fine intermetallic pinning precipitate uniformly dispersed throughout the alloy microstructure; and subsequently recrystallizing the alloy in the presence of the pinning phase to provide a grain size of ASTM 10 or finer.

45 2. The method according to claim 1 wherein: the intermetallic pinning precipitate is a spheroidal eta phase or an overaged gamma prime phase.

3. The method according to claim 2 wherein: the intermetallic pinning precipitate has an average particle size of about 0.1-1 micron.

4. The method of improving the fatigue resistance of the 50 precipitation hardenable, nickel-base alloys subject to eta phase precipitation which comprises:

55 thermomechanically processing the alloy to develop a fine spheroidal eta precipitate uniformly dispersed throughout the alloy microstructure; and subsequently recrystallizing the alloy at a temperature below the solvsus temperature of the eta precipitate to provide a grain size of ASTM 10 or finer.

5. The method according to claim 4 wherein: the thermomechanical processing comprises cold working of the alloy followed by heat treatment near but below the alloy recrystallization temperature to precipitate the spheroidal eta phase.

6. The method according to claim 4 wherein: the thermomechanical processing comprises warm working the alloy near but below the alloy recrystallization temperature to precipitate the spheroidal eta phase.

65 7. The method according to claim 4 wherein: the thermomechanical processing comprises homogenization of the alloy and precipitation of a needle-like eta phase followed by warm working near but below the alloy recrystallization temperature to convert the needle-like eta phase to the spheroidal eta phase.

70 8. The method of improving the fatigue resistance of the Inconel 718 and Incloy 901 alloys which comprises: working the alloy to effect a compressive strain equivalent

to at least a 30 percent reduction in thickness and heat treating the alloy at a temperature of 1,500°-1,750° F. to generate a fine spheroidal precipitate uniformly dispersed throughout the alloy microstructure; and subsequently recrystallizing the alloy at a temperature below the eta phase solvs to a grain size of ASTM 10 or finer.

9. The method according to claim 8 wherein: following recrystallization the alloy is heat treated to precipitate the hardening phase.
10. The method of improving the fatigue resistance of the Inconel 718 alloy which comprises: eta phase precipitation heat treatment of the homogenized alloy at 1,650°-1,700° F. for about 4-8 hours; forging to a compressive strain equivalent to at least a 30 percent reduction in thickness at a temperature of

5  
10  
15

1,750°-1,825° F. to form a fine spheroidal eta precipitate; and recrystallizing the alloy at a temperature of 1,725°-1,800° F. for about 1 hour.

11. The method of improving the fatigue resistance of the Incoloy 901 alloy which comprises: eta phase precipitation heat treatment of the homogenized alloy at 1,650°-1,700° F. for about 4-8 hours; forging to a compressive strain equivalent to at least a 30 percent reduction in thickness at a temperature of 1,700°-1,750° F. to form a fine spheroidal eta precipitate; and recrystallizing the alloy at a temperature of about 1,725°-1,750° F. for about 1 hour.

\* \* \* \* \*

20

25

30

35

40

45

50

55

60

65

70

75